

Feb. 26, 1935.

R. F. REED ET AL

1,992,771

METHOD OF PREPARING INTAGLIO LITHOGRAPHIC PLATES  
FROM ORIGINAL PLATES AND TRANSFERS

Filed Nov. 28, 1933

Fig. 1



Fig. 2



Fig. 3



Fig. 4



Fig. 5



Fig. 6



Fig. 7



Fig. 8.



INVENTORS.

Robert F. Reed  
BY Paul W. Dorst  
Anthony & George  
Wood & Wood ATTORNEYS.

Patented Feb. 26, 1935

1,992,771

# UNITED STATES PATENT OFFICE

1,992,771

## METHOD OF PREPARING INTAGLIO LITHOGRAPHIC PLATES FROM ORIGINAL PLATES AND TRANSFERS

Robert F. Reed, Paul W. Dorst, and Anthony George, Cincinnati, Ohio, assignors to The Lithographic Technical Foundation, Inc., New York, N. Y., a corporation of Delaware

Application November 28, 1933, Serial No. 700,114

8 Claims. (Cl. 41—41.5)

This invention relates to a method of preparing deep-etched or intaglio lithographic plates from original plates and transfers. As is well known in the art, lithographic plates having the design areas etched slightly below the non-printing areas may be prepared by the general method of coating the plate with a light-sensitive bichromated colloid, exposing it to light in contact with a photographic positive, dissolving the unhardened colloid from the design areas of the plate with water or other developing solution, etching the design areas slightly intaglio, depositing ink or an ink-receptive substance on the clean metal surfaces constituting the design area, and finally removing the light-hardened colloid coating from the non-printing areas. Efforts have also been made to prepare similarly deep-etched or intaglio lithographic plates from plates upon which the work has been drawn with crayon, tusche or lithographic writing ink or produced by means of hand transfers. These efforts however have not met with widespread success.

The object of this invention is to provide a method of preparing plates of this type suitable for use in the present day commercial lithographing plants. The steps in preparing plates of the type in question are as follows:

1. The design is produced upon the plate in greasy ink or crayon.
2. The plate including the design areas is coated with a powder adapted to increase the wetting action of a solution of a bichromated colloid.
3. The entire plate is coated with a solution containing a bichromated colloid.
4. The bichromated colloid is hardened by exposure to light.
5. The bichromated colloid and greasy ink are removed from the image areas.
6. The printing areas of the plate are etched slightly intaglio with an etching medium which does not attack the colloid overlying the non-design areas.
7. An ink receptive substance is deposited upon the design areas of the plate.
8. The bichromated colloid or etching resist is removed from the non-design areas.

While this series of steps summarizes the process constituting this invention, particular attention must be paid to certain important factors involved in several of the individual steps.

After the greasy printing image has been deposited upon the plate it is necessary to coat the entire plate with a material capable of forming an etching resist. A lithographic plate having a greasy design thereon presents a surface for coating that does not permit a free flow of coating solution in all directions under ordinary conditions. If coated by whirling, streaks are produced radiating from the center of rotation, by the interference of the greasy design areas with flow

of the coating solution. If the coating is done by hand as in the usual procedure of gumming up a plate, it is found that, around the boundaries of the greasy design areas, the coating is thinner than in the larger open areas and there is great difficulty in producing a coating sufficiently thick and uniform to serve as an effective etching resist.

We have found that, in a successful method of preparing deep etched plates from originals or transfers, it is necessary that the resist be capable of flowing evenly over, and coating uniformly, the greasy design areas and the non-printing areas of the plate alike. A suitable method of accomplishing this is to dust the plate with a dry powder such as rosin, asphaltum, starch, flour, talc or a mixture of two or more powders capable of adhering to the inked areas which constitute the design, and of producing capillary activity sufficient to permit free flow of the coating solution thereon.

Another point of great importance is the thickness of the film of acid resisting material. If this film be not thick enough there is a tendency for the etching acid to penetrate it and attack the non-printing areas of the plate. We have found that this drawback is overcome by using a coating solution containing more than 12 grams solids per 100 cc. and preferably about 20 grams solids per 100 cc., the exact concentration depending upon the grain of the plate and the whirler speed.

The coating solution should contain one or more proteins, such as fish glue, animal glue or albumin in combination with a bichromate. In our process we prefer a coating solution of the following composition:

|                                                                                   | Parts by weight |
|-----------------------------------------------------------------------------------|-----------------|
| Albumen (flakes)                                                                  | 1               |
| Photo-engraver's glue (50% solids)                                                | 2               |
| Ammonium bichromate                                                               | 0.6             |
| Water, sufficient to make a solution containing 20 grams total solids per 100 cc. |                 |

Good results, however, may be obtained with other proportions of the two colloids and our claims are not limited to the example given.

When the plate is coated as described above, the light-sensitive film will vary in thickness, being thicker at the boundaries of the design areas than on either the design areas or non-design areas.

The light exposure sufficient to insolubilize the bichromate colloid film of the usual thickness is insufficient to insolubilize the thicker coating existing at the design boundaries, through its entire thickness and consequently, when the ink is removed subsequently from the design areas by means of water and an ink solvent the colloid

film strips from the metal surface in the neighborhood of the design and leaves the boundaries of the design without an effective resist during the subsequent etching. This results in ragged and poorly defined design boundaries on the finished plate. We have found that it is necessary, therefore, to increase the light exposure of the bichromate-colloid film sufficiently to insolubilize those parts adjacent to the design boundaries.

10 The exposure necessary to accomplish this end is two or more times the exposure sufficient to insolubilize the colloid film not lying adjacent to the design boundaries.

It has been known to the art that light-hardened bichromate-colloid films may be removed from the plate surface through the application of either an acid or an alkali. In the case of bichromated gum arabic films, dilute solutions of mineral acids such as sulphuric acid are preferred. In the case of bichromated glue or albumen films, the preferred method of removal is the application of dilute solutions of alkali metal hydroxides. Dilute mineral acids possess the disadvantage that they rapidly attack and destroy the grain of zinc plates, reducing their water holding capacity, and also that they tend to break through the ink and attack the design areas.

Solutions of alkali metal hydroxides possess the disadvantages that (1) they rapidly attack and corrode the skin of operators and (2) they saponify and dissolve any fatty components of the ink or ink-receptive substance overlying the design. We have overcome these disadvantages by using as a remover of the bichromate-colloid film, a solution of an alkaline earth hydroxide or a mixture of an alkaline earth hydroxide and an alkaline earth salt. Such a solution does not attack the surface of zinc plates or stones, or damage the grain thereof; it is very much less corrosive to the skin of operators than solutions of alkali metal hydroxides; it does not remove the fatty components of the ink which overlies the design areas.

45 To prepare a deep-etched or intaglio lithographic plate, we proceed as follows:

An image is produced on a clean, grained zinc plate by any means in which a greasy ink or crayon is applied directly to the metal surface, such as transferring or crayon drawing, and said image is worked up in greasy ink by methods known to the art. The greasy image is then dusted first with powdered rosin and afterward with powdered talc to make the surface more easily wet by water solutions. The plate is then washed with water to remove excess rosin and talc. When the excess water has been removed but before the plate dries, it is coated with a bichromate-colloid solution preferably having the following composition:

|                                                                                   | Parts by weight |
|-----------------------------------------------------------------------------------|-----------------|
| Photo-engraver's glue (50% solids)                                                | 2               |
| Albumen (dried)                                                                   | 1               |
| 65 Ammonium bichromate                                                            | 0.6             |
| Water, sufficient to make a solution containing 20 grams total solids per 100 cc. |                 |

In order that the present invention may be better understood, reference is made to the accompanying drawing wherein:

Figure 1 is a diagrammatic elevation in section on an enlarged scale of a metal plate wherein a design has been deposited by means of greasy ink or crayon.

Figure 2 is a corresponding view showing the inked design on the metal plate covered by a rosin or talc dust.

Figure 3 is a corresponding view showing the plate after the application of the light-sensitive colloid coating.

Figure 4 shows the plate after the colloid coating has been exposed to light.

Figure 5 shows the plate after the inked design has been removed from the plate.

Figure 6 shows the plate after etching.

Figure 7 shows the plate after an ink coating has been applied after an asphaltum wash.

Figure 8 shows the plate in final form after removal of the colloid film.

The plate is whirled to distribute the coating uniformly and allowed to dry. The coated plate is next exposed to the light of an arc lamp for a period two or more times as long as is necessary to insolubilize the colloid film not adjacent to the design boundaries. After exposure the plate is washed with water, the excess water removed and, while damp, the plate is washed with a solvent for ink, such as gasoline or benzine, and rubbed gently with a cotton wad to remove the ink and its overlying film of hardened colloid. The image thus prepared is etched with a solution of an acid or salt in practically anhydrous alcohol. Acids and salts such as hydrochloric, nitric and sulphuric acid, ferric chloride, and others, are suitable for this purpose but we prefer an etch of the following composition:

Hydrochloric acid, 37%-38.5% ----- 5 cc.

Anhydrous alcohol ----- 95 cc.

The etching medium should contain a total of not more than 5% moisture. Instead of ethyl alcohol, other lower alcohols, or mixtures of two or more alcohols such as are marketed as denatured absolute alcohols may be used successfully so long as they are practically anhydrous. After etching, the plate is washed with anhydrous alcohol, gasoline or turpentine, using a wad of cotton and sufficient abrasion to dislodge the residue from the etched areas, after which the plate is dried. The plate is then coated with a solution of asphaltum or any one of the commonly used "wash-out solutions", and dried, after which it is again coated with liquid developing ink, or with a lithographic ink thinned with a solvent such as turpentine, to render the etched design greasy or grease-receptive. It is then dusted with powdered talc to render the plate surface wettable by water. The plate is then treated with a solution of the following composition:

|                                             | Grams |
|---------------------------------------------|-------|
| Barium chloride                             | 8     |
| Sodium hydroxide                            | 1     |
| Water, sufficient to make a total volume of | 60    |

100 cc.

This solution is distributed over the surface, at the same time rubbing with a wad of cotton until the colloid film is removed. The plate may or may not be counter-etched at this point by flowing with hydrochloric acid solution containing one part of 37% hydrochloric acid in 200 parts of water, but in either case it is then desensitized and rolled up in the known manner of preparing transfers or original plates for the press.

Claims directed to the use of barium chloride and barium hydroxide for removing bichromated films from lithographic plates are reserved for our co-pending application Serial Number 700,115.

Having described our invention, we desire to be limited only by the following claims:

- 5 1. A process of preparing deep-etched or intaglio lithographic plates from original plates or transfers, comprising, powdering the inked design to render it wettable, coating the entire plate with a solution of a light-sensitive bichromated protein or mixture of proteins containing more than 12 grams solids per 100 cc. of solution, exposing to light for more than double the time necessary to insolubilize the coating, removing ink from the image with an ink solvent in the presence of moisture, etching the design slightly intaglio, depositing on the design a greasy or 10 grease-receptive ground, and removing the resist by means of a solution containing an alkaline earth hydroxide.
- 15 2. A process of preparing deep-etched or intaglio lithographic plates from original plates or transfers, comprising powdering the inked design to render it wettable, coating the entire plate with a solution of a light-sensitive bichromated protein or mixture of proteins containing more than 12 grams solids per 100 cc. of solution, exposing to light for more than double the time necessary to insolubilize the coating, removing ink from the image with an ink solvent in the presence of moisture, etching the design slightly intaglio, depositing on the design a greasy or 20 grease-receptive ground, and removing the resist by means of a mixture of an alkaline earth hydroxide and an alkaline earth salt.
- 25 3. A process of preparing deep-etched or intaglio lithographic plates from original plates or transfers in which the following steps are used: dusting the inked design to render it wettable by the bichromate-colloid coating solution; coating the entire surface with a bichromate-colloid solution containing more than 12 grams 30 solids per 100 cc. of solution; exposing the bichromate-colloid coating to light for two or more times the time necessary to insolubilize the coating; removing the light-hardened colloid coating from the design area; and after etching and inking the design removing the bichromate-colloid coating with a solution containing an alkaline earth hydroxide.
- 35 4. A process of preparing deep-etched or intaglio lithographic plates from original plates or transfers in which the following steps are used: dusting the inked design to render it wettable by the bichromate-colloid coating solution; coating the entire surface with a bichromate-colloid solution containing more than 12 grams of solids 40 per 100 cc. of solution; exposing the bichromate-colloid coating to light for two or more times the time necessary to insolubilize the coating; removing the light-hardened colloid coating from the design area; and after etching and inking the design, removing the bichromate-colloid coating with a solution containing a mixture of an alkaline earth hydroxide and an alkaline earth chloride.

5 5. A process of preparing intaglio lithographic plates from original plates or transfers, comprising, coating the entire plate with a solution of a light-sensitive bichromated colloid, light-hardening the bichromated colloid over the surface of the entire plate, removing the ink and the light-hardened colloid overlying it from the printing areas of the plate by abrasion in the presence of moisture and a grease solvent, etching the printing areas of the plate slightly intaglio, depositing an ink receptive substance over the printing areas of the plate, and removing the light-hardened colloid from the non-printing areas of the plate.

10 6. A process of preparing intaglio lithographic plates from original plates or transfers, comprising, coating the entire plate with a solution of a light-sensitive mixture of glue and albumin, light-hardening the bichromated colloid over the surface of the entire plate, removing the ink and the light-hardened colloid overlying it from the printing areas of the plate by abrasion in the presence of moisture and a grease solvent, etching the printing areas of the plate slightly intaglio, depositing an ink receptive substance over 15 the printing areas of the plate, and removing the light-hardened colloid from the non-printing areas of the plate.

20 7. A process of preparing intaglio lithographic plates from original plates or transfers, comprising, coating the entire plate with a solution of a light-sensitive mixture of glue and another colloid, light-hardening the bichromated colloid over the surface of the entire plate, removing the ink and the light-hardened colloid overlying it 25 from the printing areas of the plate by abrasion in the presence of moisture and a grease solvent, etching the printing areas of the plate slightly intaglio, depositing an ink receptive substance over 30 the printing areas of the plate, and removing the light-hardened colloid from the non-printing areas of the plate.

35 8. A process of preparing intaglio lithographic plates from original plates or transfers, comprising, coating the entire plate with a solution of a light-sensitive bichromated colloid, light-hardening the bichromated colloid over the surface of the entire plate, removing the ink and the light-hardened colloid overlying it from the 40 printing areas of the plate by abrasion in the presence of moisture and a grease solvent, etching the printing areas of the plate slightly intaglio, depositing an ink receptive substance over 45 the printing areas of the plate, and removing the light-hardened colloid from the non-printing areas of the plate with a solution of alkaline earth hydroxide in water.

50 ROBERT F. REED.  
PAUL W. DORST.  
ANTHONY GEORGE.